

# United States Patent Office

2,869,995

Patented Jan. 20, 1959

1  
2,869,995

## STABILIZATION OF FUELS CONTAINING TETRAETHYL LEAD

Josef M. Michel and Karl F. Hager, Fort Bliss, Tex.,  
assignors to the United States of America as repre-  
sented by the Secretary of the Army

No Drawing. Application July 18, 1950  
Serial No. 174,567

28 Claims. (Cl. 52—5)

(Granted under Title 35, U. S. Code (1952), sec. 266)

The invention described in the specification and claims  
may be manufactured and used by or for the Government  
for governmental purposes without the payment to us  
of any royalty thereon.

It is known that tetrathyl lead either pure or mixed  
with other compounds and even when highly diluted  
as in "leaded gasoline" is not stable for any great period  
of time. It decomposes, especially when exposed to light  
or moisture, catalytically forming lead oxides and/or hydroxides.  
If equipment coming in contact with these  
decomposition products is built from copper, brass, stain-  
less steel, nickel or nickel alloys, no harmful reactions  
will take place. However, if light metals or their alloys  
are used in building such equipment, difficulties will arise  
under conditions prevailing in practical use.

By experience it has been proven that fuel containers  
made of light metals or their alloys, in particular those  
made of magnesium or magnesium alloys, will become  
perforated within a very short time when in contact with  
liquid fuels (e. g. gasoline) containing tetrathyl lead.  
Scientific investigations of this problem have lead us to  
the following explanations of the cause of the perfora-  
tion of the containers: As long as the water content of  
the liquid fuel is below the solubility limit of water in  
the fuel, there is no danger that such a formation of holes  
will take place. However, if the point is reached where  
the water is not dissolved further in the liquid fuel, but  
appears as a second or separate phase, for example, at  
the bottom of such a container, the decomposition re-  
action mentioned above will start, and eventually small  
holes passing entirely through the walls of the container  
will appear. The tetrathyl lead decomposes at the  
interface between the fuel and water, forming lead oxides  
and/or hydroxides. These compounds, having a high  
specific gravity, sink to the bottom of the container where  
they come in contact with the metal thereof and build  
up a local element of which the lead compound is the  
cathode and the magnesium alloy, the anode. This means  
that the metal of the container will dissolve. At every  
place where the decomposition products of the tetrathyl  
lead come in contact with the container walls, such an  
electrolytic corrosion starts. According to conditions, it  
may take only a very short time to produce perforations  
in the container. Tests have shown that the holes formed  
by this electrochemical process are usually found in the  
water phase or at the interface between liquid fuel and  
water. The same is true for certain other metals, for  
example, aluminum, iron, zinc, alloys of aluminum, and  
certain alloys of iron and of zinc, even if the special  
place of these metals and alloys in the electromotive  
series results in a slower action.

We have discovered that the above described decom-  
position of tetrathyl lead and the perforation of metal  
container for liquid fuels containing tetrathyl lead can  
be prevented by applying to the interior wall or walls of  
the containers, or by incorporating in or mixing with the  
liquid fuel, a hydrocarbon (alkyl)-sulfamido carboxylic  
acid or an inorganic or organic salt thereof.

2  
The said hydrocarbon-sulfamido-carboxylic acids can  
be designated by the chemical formula



5 in which  $R_1$  is an alkyl radical of at least five carbon  
atoms, and  $R_2$  an alkyl radical less one hydrogen atom.  
In other words  $R_2$  is a divalent aliphatic radical of the  
general formula  $C_nH_{2n}$  having one valency bond con-  
nected with the carbon atom of the carboxyl group and  
10 another valency bond connected with the nitrogen atom  
of the  $R_1SO_2NH$  group.  $R_1$  is preferably an alkyl radi-  
cal of from 12 to 18 carbon atoms inclusive, either of  
the straight chain or branched chain type, but preferably  
15 of the straight chain type. Examples of hydrocarbon-  
sulfamido-carboxylic acids, which may be used in the  
practice of the present invention are hydrocarbon  
( $C_{12-18}$ )-sulfamido-acetic acid; hydrocarbon ( $C_{14-16}$ )-  
sulfamido-acetic (sometimes referred to as mepasin-  
sulfamido acetic acid); octyl-sulfamido-butyric



tetradecyl-sulfamido-propionic acid,



25 and hexadecyl-sulfamido-acetic acid,



In a broader sense the hydrocarbon-sulfamido-carboxylic  
acids that may be used in the practice of the present  
invention are, or may be regarded as derivatives of the

30 lower fatty or aliphatic acids of the general formula  
 $C_nH_{2n}O_2$  such as formic acid ( $H.COOH$ ), acetic acid,  
 $CH_3COOH$ , propionic acid ( $C_2H_5COOH$ ) and butyric  
acid,  $C_3H_6COOH$ , in which a hydrogen atom thereof  
35 attached to a carbon atom has been replaced by the un-  
ivalent group  $—NHSO_2H$ ,  $R_1$  being an alkyl radical of  
the number of carbon atoms defined. The correctness  
40 of this view point arises from the fact that the hydro-  
carbon-sulfamido-carboxylic acids under consideration  
may be prepared from mono-chlor aliphatic acids by re-  
action with compounds of the type  $R_1SO_2NH_2$  with liber-  
ation of hydrogen chloride arising from one hydrogen  
45 atom of the amine group ( $NH_2$ ) of  $R_1SO_2NH_2$  uniting  
the chlorine atom of the mono-chlor aliphatic acid. As  
the chlorine atom of the mono-chlor aliphatic acid re-  
placed a hydrogen atom of the aliphatic acid, and since  
50 in the compounds under consideration the  $—NHSO_2R_1$   
group replaces the chlorine atom, the net result is, in  
effect, a replacement of a hydrogen atom (attached to  
a carbon atom) of the aliphatic acid by the  $—NHSO_2R_1$   
group. The described reaction may be conducted in the  
presence of an alkali, for example sodium or potassium  
55 hydroxide, whereby the corresponding salts of the hydro-  
carbon-sulfamido-carboxylic acid are obtained.

55 Examples of salts of hydrocarbon-sulfamido-carboxylic  
acids that may be used in practicing the invention are:  
inorganic salts such as sodium, potassium and ammonium  
salts, and salts of ammonia derivatives such as hydrazine;  
and organic salts such as salts of cyclohexylamine, methyl-  
60 yamine and ethylamine.

65 The action of these compounds is based on two funda-  
mental facts: (a) Stabilizing effect on the tetrathyl  
lead itself by inhibiting the decomposing forces of the  
humidity and the surface tension between the two phases  
when formed; and (b) formation of molecular coatings  
on the inside wall of the container that insulates the  
metal or alloy against the decomposing products of  
the tetrathyl lead, when formed occasionally, whereby  
any formation of local elements is prevented.

70 From the different actions and reactions necessary to  
satisfy these requirements and from the facts observed  
in practical use, it is easily seen that only such com-

pounds would be able to give a good and reliable protection against these electrochemical reactions that have a stabilizing effect on the lead compound and in addition a very high affinity with respect to the metal in order to be able to form films that are firmly bonded to the surface, tight, and that can not be damaged by liquid fuels, water, or diluted salts solutions.

In spite of the fact that protective coatings consisting of such metal active compounds can easily be produced by treating the metal parts with either water emulsions or organic solutions containing up to 50% hydrocarbon-sulfamido-carboxylic acids and/or their inorganic or organic salts, the simplest way and technically easiest to handle is the addition of small amounts (below 1%) of the compounds mentioned to the liquid fuels, water and diluted salt. By this method, not only the tetraethyl lead is stabilized reliably but also a protective coating is formed and even restored when damaged, e. g., by mechanical forces. Finally, the surface tension is decisively changed between the two separate phases, fuel and water, when formed.

This simple method becomes possible owing to the fact that the metal active compounds are not only soluble in the organic or liquid fuel medium but also in water.

It is known that some proposals have been made to use "mepasin"-sulfamido-acetic-acid-sodium salt as an inhibitor for fuels. From these proposals it could not be learned, predicted or foreseen at all that the process claimed and described in this application would have any stabilizing effect on tetraethyl lead and could paralyze the dangerous action of any decomposition products by forming tight coatings on the metal surface. Furthermore, no one could expect or be able to calculate theoretically in advance that a water phase originating from a fuel that contains only small amounts of hydrocarbon-sulfamido-carboxylic-acids and/or their inorganic and organic salts would dissolve any amount of metal active compound sufficiently to guarantee a reliable stabilization of the tetraethyl lead and the formation of a tight protective coating on the metal or alloy in question.

Experiments carried out as well as the methods used for proving the utility of the procedure and their results are given below:

#### Example No. 1

Welded containers made of a magnesium alloy consisting of 6.5% Al, 1.0% Zn; 0.2%, Mn; rest, magnesium. One of these was filled with a water emulsion containing 25% hydrocarbon ( $C_{12-18}$ )-sulfamido-acetic acid sodium salt at ambient temperature. After a few minutes the tank was emptied and then refilled with leaded gasoline (octane number 82). After two weeks storage, as no change in the condition of the inside walls had occurred, tap water was added in such an amount (about 1%) that a second phase was formed on the bottom of the tank. Test conditions were changed from time to time by shaking the container on a plate feeder; and by outdoor and indoor storage to get the changing ambient temperatures between day and night time. A careful check after a test period of 6 months showed no formation of local elements, either in the water or in the fuel phase, which means that the tetraethyl lead has been stabilized. In contrast, another container, same size and alloy, tested under the same conditions, but without the above described emulsion treatment showed first spots of local elements after two weeks, and after two months, it was perforated. The holes, which were substantially of microscopic size, were mostly found in the water phase, a few of them at the interface between fuel and water.

#### Example No. 2

Containers made from aluminum (99% Al; rest, iron, silicon, copper) were sprayed on the inside with a solution of 5% octyl-sulfamido-butyric acid ammonium salt in

ethyl alcohol at ambient temperature. After allowing the excess solution to drain out of the tank, it was filled with aviation gasoline (90 octane) containing tetraethyl lead and treated in the same way as mentioned for the magnesium container in Example No. 1.

While the sprayed container was entirely unchanged as to the conditions of the inside walls because of the stabilizing effect of the compound mentioned, untreated tanks showed serious corrosion symptoms caused by formation of local elements after 4 weeks only.

#### Example No. 3

Ordinary iron strips, welded, 5 x 2.5 x 0.05 inches, were put in leaded gasoline (75 octane) containing 0.05% hexadecyl-sulfamido-propionic acid cyclohexylamine salt first, without, and later on, with water forming a second phase on the bottom of the glass jars that were used for these test series. By the stabilizing effect of this compound, the results, after a period of 10 months, were excellent showing no difference on comparing the appearance of the specimens before and after storage in the leaded gasoline. On other test pieces, however, in contact with unstabilized leaded gasoline, formation of local elements could be observed appearing in rust spots, a few days after the addition of water. This reaction spread over the whole surface, first in the water, and later in the fuel phase also. After 3 months of testing by partially storing, and partially shaking, the following corrosion results were obtained:

Water phase ..... 350 g./m<sup>2</sup>  
Fuel phase ..... 160 g./m<sup>2</sup>

In comparison, the other specimens in the stabilized fuel, showed the corrosion results:

Water phase ..... 0.1 g./m<sup>2</sup>  
Fuel phase ..... 0.05 g./m<sup>2</sup>

which means an improvement ratio 1:3500.

#### Example No. 4

Fuel containers for rockets made from a magnesium alloy containing 98.5% Mg and 1.5% Mn were treated in the same way as mentioned in Example 1, using hexadecyl-sulfamido-acetic acid potassium salt as a 15% water emulsion. Aviation gasoline (92 octane) containing tetraethyl lead was the test fuel. To intensify experimentation and simulate the conditions in practical use, the fuel was changed every week. In addition, the inside wall was slightly brushed in order to remove some deposits from the bottom of the container. While no formation of local elements could be observed during the first month of testing, the stabilizing effect caused by the hydrocarbon-sulfamido-carboxylic-acid film decreased remarkably afterwards, and 10 days later (about 40 days after starting the test) formation of local elements followed by electrochemical reactions had already started at several places.

In order to avoid these difficulties it was found that it is sufficient to add small amounts of the metal active compound in question to the fuel. By doing so, it was observed not only that the decomposition of the tetraethyl lead was stopped but also that the damaged coating was restored at once, even if the weak spots were situated in the water phase.

According to this result, other containers, same shape and alloy, were handled in this way, that 0.05% hexadecyl sulfamido acetic acid potassium salt were added to the test gasoline and then the same test procedure was observed as mentioned above. Even after a period of 8 months, all the containers were in excellent condition and not a single spot of attack caused by deposit of lead oxides on the inside wall, especially in the water phase or at the interface between fuel and water, could be found.

## Example No. 5

A feeding system of the type and specification as used in rockets and ramjets, consisting of pipelines, valves, pumps, containers and additional fittings and made of different metals and alloys (iron, aluminum, and magnesium alloys, stainless steel, brass, etc.), was tested with different fuel mixtures containing tetraethyl lead with and without addition of hydrocarbon ( $C_{12-18}$ ) sulfamido acetic acid sodium salt. It was found that only when using emulsions or solutions of the metal active compounds mentioned for the pre-treatment of the system or by addition of small amounts (below 1%) of those chemicals to the fuel or fuel mixtures in question, it was possible by stabilization of the tetraethyl lead to avoid any chemical or electrochemical action with the feeding system. This is especially true when the feeding system was cleaned mechanically and rinsed with water between two test runs in order to remove fuel residues.

In all other cases, using fuel compositions without additional admixtures of stabilizing and metal active compounds like hydrocarbon - sulfamido - carboxylic - acids and/or their inorganic and/or organic salts formation of local elements or electrochemical reactions started after a short time, especially on the light metal parts which are more endangered according to their position in the electromotive series.

With fuels and fuel mixtures containing even very small amounts of the metal active compounds mentioned above, it was possible to operate such systems for months without any trouble in spite of the fact that not only the fuels and fuel mixtures but also the structure and assembly of the whole equipment were changed several times, according to the special demands of the tests in question.

We claim:

1. The method of protecting a metallic surface exposed to contact with a fuel composition consisting of a water-containing gasoline carrying tetraethyl lead, said fuel composition being normally corrosive to said metallic surface, which comprises supplying to said metallic surface from 0.05% to an amount below 1% of a stabilizing agent dispersed in gasoline, said stabilizing agent being selected from the group consisting of an organic compound having the formula



in which  $R_1$  is an alkyl radical of from 5 to 18 carbon atoms and  $R_2$  is a lower aliphatic radical of the general formula  $C_nH_{2n}$  where  $n$  is a small positive integer, and the salts of said organic compound taken from the group consisting of sodium, potassium, ammonium, hydrazine, cyclohexylamine, methylamine, ethylamine and mixtures thereof, and acting on said metallic surface with said stabilizing agent to stabilize and protect said surface against the corrosive action of said fuel composition.

2. The method according to claim 1 wherein the stabilizing agent is mepasin-sulfamido-acetic acid sodium salt.

3. The method according to claim 1 wherein the stabilizing agent is octyl-sulfamido-butyric acid ammonium salt.

4. The method according to claim 1 wherein the stabilizing agent is tetradecyl-sulfamido-propionic acid cyclohexylamine salt.

5. The method according to claim 1 wherein the stabilizing agent is hexadecyl-sulfamido-acetic acid potassium salt.

6. The method according to claim 1 wherein the stabilizing agent is a sulfamido-acetic acid sodium salt of a saturated hydrocarbon.

7. The method according to claim 1 wherein the supplied stabilizing agent is in amount in excess of that required to stabilize the metallic surface, and the surface is subsequently contacted with a gasoline fuel containing tetraethyl lead.

8. The method of protecting a metallic surface exposed to contact with a fuel composition consisting of a water-containing gasoline and tetraethyl lead, said fuel composition being normally corrosive to said metallic surface, which comprises supplying to said metallic surface a stabilizing agent dispersed in an inert solvent, said stabilizing agent being selected from the group consisting of an organic compound having the formula



in which  $R_1$  is an alkyl radical of from 5 to 18 carbon atoms and  $R_2$  is a lower aliphatic radical of the general formula  $C_nH_{2n}$  where  $n$  is a small positive integer, and the salts of said organic compound taken from the group consisting of sodium, potassium, ammonium, hydrazine, cyclohexylamine, methylamine, ethylamine and mixtures thereof, said stabilizing agent being present in said inert solvent from 0.05% to an amount below 1%.

9. A method of protecting a metallic surface exposed to contact with a fuel composition consisting of water, ethyl alcohol and leaded gasoline, said fuel composition being normally corrosive to said metallic surface, which comprises supplying to said metallic surface a stabilizing agent dispersed in said fuel composition and constituting from 0.05% to an amount below 1% thereof, said stabilizing agent being selected from the group consisting of an organic compound having the general formula



in which  $R_1$  is an alkyl radical of from 15 to 18 carbon atoms and  $R_2$  is a lower aliphatic radical of the general formula  $C_nH_{2n}$  where  $n$  is a small positive integer, and the salts of said organic compound taken from the group consisting of sodium, potassium, ammonium, hydrazine, cyclohexylamine, methylamine, ethylamine and mixtures thereof, and acting on said metallic surface with said stabilizing agent to stabilize and protect said surface against the corrosive action of said fuel composition.

10. The method according to claim 9 wherein the stabilizing agent is mepasin-sulfamido-acetic acid sodium salt.

11. The method according to claim 9 wherein the stabilizing agent is acetyl-sulfamido-butyric acid ammonium salt.

12. The method according to claim 9 wherein the stabilizing agent is tetradecyl-sulfamido-propionic acid cyclohexylamine salt.

13. The method according to claim 9 wherein the stabilizing agent is hexadecyl-sulfamido-acetic acid potassium salt.

14. The method according to claim 9 wherein the stabilizing agent is hydrocarbon sulfamido-acetic acid sodium salt.

15. The method according to claim 9 wherein the supplied stabilizing agent is in an amount in excess of that required to stabilize the metallic surface and the surface is subsequently contacted with said fuel composition.

16. A composition of matter consisting essentially of leaded gasoline carrying water and from 0.05% to an amount below 1% of a stabilizing agent dispersed in an inert solvent, said stabilizing agent being taken from the class consisting of an organic compound having the formula  $R_1-SO_2-NH-R_2-COOH$  in which  $R_1$  is an alkyl radical of from 5 to 18 carbon atoms and  $R_2$  is a lower aliphatic radical of the general formula  $C_nH_{2n}$  where  $n$  is a small positive integer, and the salts of said organic compound taken from the group consisting of sodium, potassium, ammonium, hydrazine, cyclohexylamine, methylamine, ethylamine and mixtures thereof.

17. A composition according to claim 16 wherein the stabilizing agent is mepasin-sulfamido-acetic acid sodium salts.

18. A composition according to claim 16 wherein the stabilizing agent is octyl sulfamido-butyric acid ammonium salt.

19. A composition according to claim 16 wherein the stabilizing agent is tetraethyl-sulfamido-propionic cyclohexylamine salt.

20. A composition according to claim 16 wherein the stabilizing agent is hexadecyl-sulfamido acetic acid potassium salt.

21. A composition according to claim 16 wherein the stabilizing agent is a sulfamido-acetic acid sodium salt of a saturated hydrocarbon.

22. A fuel consisting essentially of gasoline, tetraethyl lead and from 0.05% to an amount below 1% of an added compound selected from the group consisting of an organic compound having the general formula



in which  $R_1$  is an alkyl radical of from 5 to 18 carbon atoms and  $R_2$  is a lower aliphatic radical of the general formula  $C_nH_{2n}$  where  $n$  is a small positive integer, and the salts of said organic compound taken from the group consisting of sodium, potassium, ammonium, hydrazine, cyclohexylamine, methylamine, ethylamine and mixtures thereof.

5

10

15

20

23. The fuel of claim 22 in which the added compound is mepasin-sulfamido-acetic acid sodium salt.

24. The fuel of claim 22 in which the added compound is octyl-sulfamido-acetic acid ammonium salt.

25. The fuel of claim 22 in which the added compound is tetradecyl-sulfamido-propionic acid cyclohexylamine salt.

26. The fuel of claim 22 in which the added compound is hexadecyl-sulfamido-acetic acid potassium salt.

27. The fuel of claim 22 in which the fuel contains water.

28. The fuel of claim 22 in which the added compound is a sulfamido-acetic acid sodium salt of a saturated hydrocarbon.

References Cited in the file of this patent

UNITED STATES PATENTS

|           |               |               |
|-----------|---------------|---------------|
| 2,183,856 | Meyer         | Dec. 19, 1939 |
| 2,578,725 | Michel et al. | Dec. 18, 1951 |
| 2,680,066 | Michel et al. | June 1, 1954  |